

## [54] IMAGE-RECEIVING ELEMENTS

[75] Inventors: Irena Y. Bronstein-Bonte, Newton; Edward P. Lindholm, Boston; Lloyd D. Taylor, Lexington, all of Mass.

[73] Assignee: Polaroid Corporation, Cambridge, Mass.

[21] Appl. No.: 143,281

[22] Filed: Apr. 24, 1980

[51] Int. Cl.<sup>3</sup> ..... G03C 5/54; G03C 1/40

[52] U.S. Cl. ..... 430/213; 430/215; 430/216; 430/221; 430/236; 430/237

[58] Field of Search ..... 430/214, 215, 216, 221, 430/227, 236, 237, 244, 213; 428/484, 515, 522

## [56] References Cited

## U.S. PATENT DOCUMENTS

3,698,896 10/1972 Abbott ..... 430/213

|           |         |                  |         |
|-----------|---------|------------------|---------|
| 3,706,557 | 12/1972 | Arond .....      | 430/215 |
| 3,734,727 | 5/1973  | Milligan .....   | 430/216 |
| 3,778,265 | 12/1973 | Land .....       | 430/213 |
| 3,930,864 | 1/1976  | Abel et al. .... | 430/213 |
| 4,190,447 | 2/1980  | Coil et al. .... | 430/215 |

Primary Examiner—Richard L. Schilling  
Attorney, Agent, or Firm—Stanley H. Mervis

## [57] ABSTRACT

Diffusion transfer films and processes are disclosed wherein the processing composition includes a light-reflecting pigment and an optical filter agent, and the image-receiving layer carries over it a layer containing a substantially non-diffusible agent adapted to decolorize optical filter agent immediately adjacent the interface between said processing composition and said decolorizing layer.

11 Claims, 1 Drawing Figure





## IMAGE-RECEIVING ELEMENTS

This invention is concerned with photography and, more particularly, with photographic processes which are conducted outside of the camera in which the film is exposed.

U.S. Pat. No. 3,415,644 issued Dec. 10, 1958 to Edwin H. Land discloses photographic products and processes wherein a photosensitive element and an image-receiving element are maintained in fixed relationship prior to exposure, and this relationship is maintained as a laminate after processing and image formation. In these products and processes, the final image is viewed through a transparent (support) element against a reflection, i.e., white, background. Photoexposure is made through said transparent element and application of the processing composition provides a layer of light-reflecting material to provide a white background for viewing the final image through said transparent support. The light-reflecting material (referred to in said patent as an "opacifying agent") is preferably titanium dioxide, and it also performs an opacifying function, i.e., it is effective to mask the developed silver halide emulsions so that the transfer image may be viewed without interference therefrom, and it also helps to protect the photoexposed silver halide emulsions from post-exposure fogging by light passing through said transparent layer if the photoexposed film unit is removed from the camera before image-formation is completed.

U.S. Pat. No. 3,647,437, issued Mar. 7, 1972 to Edwin H. Land, discloses photographic products which may be processed outside of the camera in which the film is exposed, fogging of the film by ambient light being prevented by provision of one or more opacifying dyes, sometimes referred to as light-absorbing optical filter agents, appropriately positioned in the film unit after photoexposure. In a particularly useful embodiment of that invention, the film unit is a film unit of the type described in the aforementioned U.S. Pat. No. 3,415,644 and comprises first and second sheet-like elements, the first sheet-like element comprising an opaque base carrying a silver halide emulsion, and the second sheet-like element comprising a transparent support carrying an image layer, i.e., a layer adapted to receive an image-wise distribution of an image-forming material initially present in said first sheet-like element. After photoexposure a processing composition, adapted to develop the exposed silver halide emulsion and to form the desired image in said image layer, is distributed in a thin layer between said sheet-like elements. The processing composition contains a light-reflecting pigment, such as titanium dioxide, and at least one light-absorbing optical filter agent, such as a pH-sensitive phthalein dye which is colored at the initial pH of said processing composition. As disclosed in said U.S. Pat. No. 3,647,437, the concentrations of said light-reflecting pigment and said optical filter agent(s) are such that the layer of processing composition is sufficiently opaque to light actinic to the silver halide emulsion that the film unit may be ejected from the camera immediately after the processing composition is distributed, notwithstanding the fact that the second sheet-like element will transmit light incident on the surface thereof. This opacification system is quite effective and is employed in Polaroid Land SX-70 film. The light-absorbing capacity of the optical filter agent is discharged after this ability is no longer needed, so that the optical filter agent need not be re-

moved from the film unit. Where the optical filter agent is a pH-sensitive dye, such as a phthalein indicator dye, it may be discharged or decolorized by reducing the pH after a predetermined time, e.g., by making available an acid-reacting material such as a polymeric acid.

In the preferred embodiments of the opacification system described in U.S. Pat. No. 3,647,437 the concentrations of the light-reflecting pigment and light-absorbing optical filter agent in the layer of processing composition will be such that that layer will have a transmission density of at least about 6 but a reflection density not greater than about 1. The presence of a long chain substituent, e.g., a long chain alkoxy group, on the optical filter agent is useful in reducing its diffusibility so that diffusion to the image-receiving layer is minimized.

A reflection density of about 1 will be recognized as very small compared with a transmission density of 6 or more for the same layer. In practice it has been possible to use a concentration of optical filter agents and titanium dioxide such that the reflection density of the processing composition layer, as measured about 30 seconds after distribution, is much lower than 1, e.g., about 0.5 to 0.6. While transferring dye and the emerging dye image may be seen at opacification system reflection densities of about 0.5, the presence of such temporary coloration of the highlight or white areas of the image, and the temporary distortion of the colors of the already transferring image dyes, is aesthetically undesirable.

As noted above, where the optical filter agent is a pH-sensitive dye, it is "discharged", i.e., rendered substantially colorless, by a reduction of the pH of the strata containing the optical filter agent. These strata include the light-reflecting pigment layer, provided by the processing composition, as well as the image-receiving layer and any other layers between the light-reflecting pigment layer and the transparent support through which the final image is viewed. This pH reduction is effected, to a pH level below the pKa of the optical filter agent, after a predetermined time. This delay is necessary in order that silver halide development be substantially completed before incident light is transmitted to the developing silver halide emulsions. Since the image dyes are preferably soluble and diffusible at the initial pH of the process but substantially nondiffusible at a lower pH, reduction of the pH to the appropriate lower pH after a predetermined period serves the very important function of controlling unwanted continued transfer of image dyes after the desired dye image has been formed.

It will be recognized that these desired results of pH reduction are only partly compatible, for early pH reduction to provide a white background early in the process could prematurely stop transfer of image dyes, resulting in a pale, i.e., low density, image which may also have an unbalanced color balance.

The copending application of Edwin H. Land, Leon D. Cerankowski and Neil Mattucci, Ser. No. 33,001, filed Apr. 24, 1979 (now abandoned and replaced by a continuation-in-part thereof, Ser. No. 143,293 filed Apr. 24, 1980), discloses and claims diffusion transfer products and processes of the foregoing type where the background appears substantially white to the viewer, substantially immediately after the processing composition is applied while retaining opacification. As disclosed in said application, it has been found that it is possible to significantly reduce the reflection density provided by the layer of processing composition con-

taining the light-reflecting pigment and the optical filter agent without significantly reducing the transmission density thereof. This highly desirable improvement is obtained by decolorizing, substantially immediately after application of the processing composition, the optical filter agent immediately adjacent the interface between the processing composition and the layer of the second sheet-like element in contact with the processing composition. It is only necessary to decolorize a very small fraction of the applied optical filter agent in order to effectively render the interface substantially "white" when viewed by reflection. Since the reflection density is the result of light being absorbed twice by a given quantity of dye—once when the light enters and a second time when it is reflected back—it will be seen that decolorization of even a few molecules of dye adjacent the interface provides an effect which is so amplified by the optics of reflection that one can substantially lower the reflection density and increase the apparent whiteness of the layer of the processing composition providing the background against which the image is viewed without reducing the transmission density of the "white" layer to any significant extent.

The "decolorizing" layer is provided between the image-receiving layer and the layer of processing composition. This decolorizing layer comprises a substantially nondiffusible agent adapted to decolorize the small concentration of optical filter agent which is present immediately adjacent the interface between the processing composition and the decolorizing layer. This decolorizing is essentially limited to the optical filter agent which is present immediately adjacent the interface between the decolorizing layer and the processing composition. Even though the decolorizing layer is relatively thin it inhibits diffusion of optical filter agent into the image-receiving layer where it may react with the mordant to form a "new species" whose color is discharged only at a lower pH; e.g., the new species exhibits a much lower pKa and remains colored until the pH is reduced to a much lower level than otherwise would be required for decolorization. The remaining optical filter agent is discharged or decolorized by a subsequent pH reduction.

In the preferred embodiments, the decolorizing agent is a polyoxyalkylene polymer and the optical filter agent is a pH-sensitive phthalein dye. Such polyoxyalkylene polymers tend to be "soft" or waxy materials, tend to rub off or to "block" when the sheet is rolled up and be pulled off when the sheet is unrolled.

The present invention provides decolorizing layers containing polyether, i.e., polyoxyalkylene polymers which layers are "hard" and exhibit good adhesion to the image-receiving layer of the image-receiving element. In accordance with the present invention, the decolorizing layer comprises a polyoxyalkylene polymer hydrogen-bonded to another polymer to provide a "hard" decolorizing layer.

As indicated above, this invention is primarily directed to photographic processes wherein the desired image is obtained by processing an exposed photosensitive silver halide material, with a processing composition distributed between two sheet-like elements, one of said elements including said photosensitive material. The processing composition is so applied and confined within and between the two sheet-like elements as not to contact or wet outer surfaces of the superposed elements, thus providing a film unit or film packet whose external surfaces are dry. The processing composition is

viscous and preferably is distributed from a single-use rupturable container; such pressure rupturable processing containers are frequently referred to as "pods". The final image may be black-and-white, monochrome or multicolor and either negative or positive with respect to the photographed subject. The present invention is especially, if not uniquely, adapted for facilitating processing outside of a camera film units which are maintained as an integral laminate after processing, the desired image being viewed through one face of said laminate.

In diffusion transfer embodiments of this invention the diffusible image-providing substance may be a complete dye or a dye intermediate, e.g., a color coupler. The preferred embodiments of this invention use a dye developer, that is, a compound which is both a silver halide developing agent and a dye disclosed in U.S. Pat. No. 2,983,606, issued May 9, 1961 to Howard G. Rogers. As is now well known, the dye developer is immobilized or precipitated in developed areas as a consequence of the development of the latent image. In unexposed and partially exposed areas of the emulsion, the dye developer is unreacted and diffusible and thus provides an imagewise distribution of unoxidized dye developer, diffusible in the processing composition, as a function of the point-to-point degree of exposure of the silver halide emulsion. At least part of this imagewise distribution of unoxidized dye developer is transferred, by imbibition, to a superposed image-receiving layer to provide a reversed or positive color image of the developed image. The image-receiving layer preferably contains a mordant for transferred unoxidized dye developer. As disclosed in the aforementioned U.S. Pat. Nos. 2,983,606 and 3,415,644, the image-receiving layer need not be separated from its superposed contact with the photosensitive element, subsequent to transfer image formation, if the support for the image-receiving layer, as well as any other layers intermediate said support and image-receiving layer, is transparent and a processing composition containing a substance, e.g., a white pigment, effective to mask the developed silver halide emulsion or emulsions is applied between the image-receiving layer and said silver halide emulsion or emulsions.

Dye developers, as noted above, are compounds which contain, in the same molecule, both the chromophoric system of a dye and also a silver halide developing function. By a "silver halide developing function" is meant a grouping adapted to develop exposed silver halide. A preferred silver halide development function is a hydroquinonyl group.

Multicolor images may be obtained using the color image-forming components, for example, dye developers, in an integral multi-layer photosensitive element, such as is disclosed in the aforementioned U.S. patents and in U.S. Pat. No. 3,345,163 issued Oct. 3, 1967 to Edwin H. Land and Howard G. Rogers. A suitable arrangement of this type comprises a support carrying a red-sensitive silver halide emulsion stratum, a green-sensitive silver halide emulsion stratum and a blue-sensitive silver halide emulsion stratum, said emulsions having associated therewith, respectively, for example, a cyan dye developer, a magenta dye developer and a yellow dye developer. The dye developer may be utilized in the silver halide emulsion stratum, for example in the form of particles, or it may be disposed in a stratum (e.g., of gelatin) behind the appropriate silver halide emulsion stratum. Each set of silver halide emulsion

and associated dye developer strata preferably are separated from other sets by suitable interlayers. In certain instances, it may be desirable to incorporate a yellow filter in front of the green-sensitive emulsion and such yellow filter may be incorporated in an interlayer. However, if the yellow dye developer has the appropriate spectral characteristics and is present in a state capable of functioning as a yellow filter, a separate yellow filter may be omitted.

For convenience, further description of this invention will be in the context of the use of dye developers and positive transfer images. Also for convenience, the disclosure of the aforementioned copending application, Ser. No. 33,001, now abandoned, is expressly incorporated herein.

Referring to the FIGURE, Stages A, B and C show in diagrammatic cross-section, respectively, imaging, processing, and the finished print in one embodiment of this invention. For ease of understanding, the FIGURE illustrates the formation of a monochrome image using a single dye developer. In Stage A, there is shown a photosensitive element 30 in superposed relationship with an image-receiving element 32, with a rupturable container 16 (holding an opaque processing composition 17) so positioned as to discharge its contents between said elements upon suitable application of pressure, as by passing through a pair of pressure applying rolls or other pressure applying means (not shown). Photosensitive element 30 comprises an opaque support 10 carrying a layer 12 of a dye developer over which has been coated a silver halide emulsion layer 14. The image-receiving element 32 comprises a transparent support 24 carrying, in turn, a polymeric acid layer 22, a spacer layer 20, an image-receiving layer 18 and a decolorizing layer 26. Photoexposure of the silver halide emulsion layer is effected through the transparent support 24 and the layers carried thereon, i.e., the polymeric acid layer 22, the spacer layer 20, the image-receiving layer 18 and the decolorizing layer 26, which layers are also transparent, the film unit being so positioned within the camera that light admitted through the camera exposure or lens system is incident upon the outer or exposure surface 24a of the transparent support 24. After exposure the film unit is advanced between suitable pressure-applying members, rupturing the container 16, thereby releasing and distributing a layer 17a of the opaque processing composition and thereby forming a laminate, as illustrated in processing Stage B, of the photosensitive element 30 and the image-receiving element 32 with their respective support members providing the outer layers of the laminate (illustrated in Stage B). The opaque processing composition contains a film-forming polymer, a white pigment and has an initial pH at which one or more optical filter agents contained therein are colored; the optical filter agent (agents) is (are) selected to exhibit the appropriate light absorption, i.e., optical density, over the wavelength range of light actinic to the particular silver halide emulsion(s). As a result, ambient or environmental light within that wavelength range incident upon transparent support surface 24a and transmitted transversely through said transparent support and the transparent layers carried thereon in the direction of the exposed silver halide emulsion 14a is absorbed thereby avoiding further exposure of the photoexposed and developing silver halide emulsion 14a. In exposed and developed areas, the dye developer is oxidized as a function of the silver halide development and immobilized. Unoxidized

dye developer associated with undeveloped and partially developed areas remains mobile and is transferred imagewise to the image-receiving layer 18 to provide the desired positive image therein. Permeation of the 5 alkaline processing composition through the image-receiving layer 18 and the spacer layer 20 to the polymeric acid layer 22 is so controlled that the process pH is maintained at a high enough level to effect the requisite development and image transfer and to retain the 10 optical filter agent (agents) in colored form within the processing composition layer 17a and on the silver halide emulsion side of said layer 17a, after which pH reduction effected as a result of alkali permeation into the polymeric acid layer 22 is effective to reduce the pH 15 to a level which changes the optical filter agent to a colorless form. Absorption of the water from the applied layer 17a of the processing composition results in a solidified film composed of the film-forming polymer and the white pigment dispersed therein, thus providing reflecting layer 17b which also serves to laminate together the photosensitive component 30 and the image-receiving component 32 to provide the final laminate (Stage C). The positive transfer image in dye developer present in the image-receiving layer 18a is viewed through the transparent support 24 and the intermediate transparent layers against the reflecting layer 17b which provides an essentially white background for the dye image and also effectively masks from view the developed silver halide emulsion 14b and dye developer immobilized therein or remaining in the dye developer layer 12.

The optical filter agent is retained within the final film unit laminate and is preferably colorless in its final form, i.e., exhibiting no visible absorption to degrade 35 the transfer image or the white background therefor provided by the reflecting layer 17b. The optical filter agent may be retained in the reflecting layer under these conditions, and it may contain a suitable "anchor" or "ballast" group to prevent its diffusion into adjacent 40 layers. Some of the optical filter agent may diffuse into the photosensitive component and be mordanted by the gelatin or other material present on the silver halide emulsion side of the reflecting layer 17b; optical filter mordanted in the photosensitive component 30 may be 45 colorless or colored in its final state so long as any color exhibited by it is effectively masked by the reflecting layer 17b. In a preferred embodiment, the image-receiving element is free of gelatin; the photosensitive element contains gelatin, and the optical filter agent(s) is a pH-sensitive phthalein dye.

In the illustrated embodiment, photoexposure is effected through the image-receiving element. While this is a particularly useful and preferred embodiment, especially where the photosensitive element and the image-receiving element are secured together as shown in U.S. Pat. Nos. 3,415,644 and 3,647,437, it will be understood that the image-receiving element may be initially positioned out of the exposure path and superposed upon the photosensitive element after photoexposure.

A light-absorbing material optical filter agent, preferably a pH-sensitive dye such as an indicator dye, is provided so positioned and/or constituted as not to interfere with photoexposure but so positioned between the photoexposed silver halide emulsions and the transparent support during processing after photoexposure 65 as to absorb light which otherwise might fog the photoexposed emulsions. Furthermore, the light-absorbing material is so positioned and/or constituted after pro-

cessing as not to interfere with viewing the desired image shortly after said image has been formed. In the preferred embodiments, the optical filter agent is initially contained in the processing composition in colored form together with a light-reflecting material, e.g., 5 titanium dioxide.

The concentration of indicator dye is selected to provide the optical transmission density required, in combination with other layers intermediate the silver halide emulsion layer(s) and the incident radiation, to 10 prevent nonimagewise exposure, i.e., fogging, by incident actinic light during the performance of the particular photographic process. The transmission density and the indicator dye concentration necessary to provide the requisite protection from incident light may be 15 readily determined for any photographic process by routine experimentation, as a function of film speed or sensitivity, processing time, anticipated incident light intensity, etc., as described in said U.S. Pat. No. 3,647,437. It will be recognized that a particular transmission density may not be required for all portions of the spectrum, lesser density being sufficient in wavelength regions corresponding to lesser sensitivities of the particular photosensitive material.

In a particularly useful embodiment, the light-absorbing dye is highly colored at the pH of the processing composition, e.g., 13-14, but is substantially non-absorbing of visible light at a lower pH, e.g., less than 10-12. Particularly suitable are phthalein dyes having a pKa of about 13 to 13.5; many such dyes are described in the aforementioned U.S. Pat. No. 3,647,437. This pH reduction may be effected by an acid-reacting reagent appropriately positioned in the film unit, e.g., in a layer 20 between the transparent support and the image-receiving layer, as described in more detail below.

It will be understood that a mixture of light-absorbing materials may be used so as to obtain absorption in all critical areas of the visible and near-visible by which the silver halide emulsions, e.g., a panchromatic black-and-white silver halide emulsion or a multicolor silver halide photosensitive element, being used are exposable. Many dyes which change from colored to colorless as a function of pH reduction, e.g., phthalein dyes, are known and appropriate selection may be made by one skilled in the art to meet the particular conditions of a 45 given process and film unit; such dyes are frequently referred to in the chemical and related arts as indicator dyes.

In accordance with this invention the optical filter agent(s) is a pH-sensitive phthalein dye and the decolorizing agent is a polyether, i.e., a polyoxyalkylene polymer, coated with another polymer which can form a 50 hydrogen bond complex with the polyether to provide a decolorizing layer which is sufficiently "hard" to resist rub off and blocking.

The polyether should be substantially non-diffusible from the decolorizing layer into the processing composition, thereby avoiding premature discharge of the optical filter agent in the processing composition layer. This factor may be controlled by selecting a higher 60 molecular weight polyether or by selecting a polyether having a sufficient hydrocarbon group to reduce its diffusibility. The polyether should not be a liquid at room temperature. The preferred polyethers are waxes at room temperature.

The ability of a given polyether to decolorize the particular optical filter agent(s) may be readily determined by a procedure such as the following: the optical

filter agent in question is dissolved in 1.5 molar aqueous potassium hydroxide to provide a solution of about 0.01 weight percent of the optical filter agent in a test tube. The test decolorizing agent is added to the test tube in small increments. Decolorizing agents which decolorize or substantially reduce the visible absorption of the optical filter agent when added to the potassium hydroxide in quantities less than about 35 times (by weight) the optical filter agent concentration in said solution are preferred as they avoid the need to use undesirably high decolorizing layer coverages, e.g., such thickness as might undesirably slow down or reduce the transfer of image dye.

As examples of polyethers useful in this invention, mention may be made of the polyoxyethylene polyoxypropylene block copolymer commercially available under the tradename "Pluronic F-127" from BASF Wyandotte Corp. (average molecular weight about 12,500) and the nonylphenyl terminated polyoxyethylene



sold under the tradename "Igepal CO-890" by GAF.

As noted in the aforementioned copending application Ser. No. 33,001, now abandoned, Pluronic F-127 has been found effective with a number of phthalein dyes. Igepal CO-890 has been found to be at least as effective as Pluronic F-127, and to be more effective in decolorizing phthalein dyes such as:



The mechanism by which the decolorization occurs using the polyether is not a pH change. It has been determined that the addition of either Igepal CO-890 or Pluronic F-127 did not change the pH. It appears that the presence of a long chain substituent on the phthalein dye markedly reduces the quantity of the polyether required to effect the decolorization. It is believed that the polyether forms a complex with the phthalein dye which complex exhibits an apparent pKa higher than said phthalein dye in the alkaline processing composition. It also appears that phthalein dyes containing the grouping



are more readily decolorized by the polyether.

As noted above, use of a polyoxyethylene polyoxypropylene block copolymer has been found to be useful in the practice of this invention. Such block copolymers may be represented by the formula



Varying the ratios  $a$ ,  $b$  and  $c$  will vary the hydrophobic-hydrophilic balance of the block copolymer and such varying may be of value in the practice of this invention. Other polyoxyalkylene polymers, such as high molecular weight polyethylene glycol (m.wt. 6000) commercially available under the tradename Carbowax 6000 also may be used, although the above block copolymers are more effective.

A particularly effective polymer hydrogen bonding a polyether decolorizing agent is a copolymer of diacetone acrylamide and methacrylic acid, preferably a 1:1 monomer ratio. Hydrogen bonding—a non-valent bonding—is believed to occur between the  $-\text{COOH}$  groups provided by the methacrylic acid and the oxygen of the ether group ( $-\text{CH}_2-\text{CH}_2-\text{O}-\text{CH}_2-\text{CH}_2-$ ). The diacetone acrylamide provides a hydrophobic property, and the ratio of the two monomers may be adjusted to provide the balance of hydrophilic and hydrophobic properties desired for a given photographic system. 1:1 copolymers of methacrylic acid and diacetone acrylamide having a molecular weight of about 10,000 to 20,000 have been found to be particularly useful. The polymeric polyether preferably has a molecular weight of at least about 2000; the molecular weight in combination with the hydrophilic/hydrophobic properties of the polymeric polyether should be such as to render it substantially nondiffusible from the decolorizing layer. Where the ether groups do not hydrogen bond with sufficient  $-\text{COOH}$  groups to give the desired "hardness", e.g., because the molecular geometry does not provide the appropriate "fit", another hydrogen bonding polymer, e.g., polyvinyl pyrrolidone, may be incorporated. Hydrogen bonding also may occur between the carboxyl group and the amide groups. The particular hydrogen bonding group is not important, and suitable materials may be readily selected by routine experimentation. The hydrogen bonded complex should precipitate in water. The hydrogen bond is reversible in aqueous alkaline solution, thus making the polyether decolorizing agent available to complex with the phthalein optical filter agent and to permit rapid diffusion of the image dye (s) through the decolorizing layer to the image-receiving layer.

As noted above, methacrylic acid is a preferred monomer in the hydrogen bonding polymer. Acrylic acid also may be used but is a less effective hydrogen bonding agent, possibly because fewer carboxyl groups are properly positioned to hydrogen bond with the polyether. The pendant methyl groups of the methacrylic acid moieties are believed to limit the ability of the carboxyl group to rotate around the polymer backbone, so that more of the carboxyl groups are properly positioned.

In the preferred embodiment of this invention the decolorizing layer comprises a mixture of a 1:1 diacetone acrylamide/methacrylic acid copolymer, the 65 nonyl phenol meno ether of a polyethylene glycol ( $n=40$ ) (Igepal CO-890), and a low molecular weight polyvinyl pyrrolidone, e.g., "PVP K-30" polyvinyl

pyrrolidone having a molecular weight of about 15,000 and commercially available from GAF Corporation. Suitable ratios of these components, respectively, include 1.0/1.0/0.35 and 1.0/0.75/0.35 parts by weight.

5 Such mixtures may be coated at a coverage of about 50 to 100 mg./ft.<sup>2</sup> (about 538 to 1076 mg./m<sup>2</sup>). Suitable coating solvents include aqueous ethanol, to which may be added a ketone such as methyl ethyl ketone. The solvent system should be selected to avoid having an 10 adverse effect upon the image-receiving layer and to minimize the formation of haze. Examples of suitable solvent systems for coating such decolorizing layers include (by volume) (1) and 80/20 water/ethanol mixture and (2) 50/35/15 acetone, ethanol and water. The 15 DAA/MAA copolymer is added as the ammonium salt, with the free acid being regenerated during drying by volatilization of ammonia.

The following examples of image-receiving elements employing decolorizing layers in accordance with this invention are intended to be illustrative and are not intended to be limiting. All parts and percentages are by weight unless otherwise stated.

#### EXAMPLE 1

An image-receiving element was prepared by coating a transparent polyethylene terephthalate 4 mil (0.1 mm) support with the following layers:

20 1. a neutralizing layer comprising approximately 9 parts of a half-butyl ester of polyethylene/maleic anhydride and 1 part of polyvinyl butyral coated at a coverage of about 2500 mg./ft<sup>2</sup> (about 26,900 mg./m<sup>2</sup>);

25 2. a timing layer comprising about 270 mg./ft<sup>2</sup> (about 2900 mg./m<sup>2</sup>) of a 60.6/29/6.3/3.7/0.4 pentapolymer of butylacrylate, diacetone acrylamide, styrene, methacrylic acid and acrylic acid and about 30 mg./ft<sup>2</sup> (about 320 mg./ft<sup>2</sup> of polyminyl alcohol;

30 3. an image-receiving layer coated at a coverage of about 300 mg./ft<sup>2</sup> (about 3330 mg./m<sup>2</sup>) of a mixture of 3 parts of (a) a 2:1 mixture of polyvinyl alcohol and poly-4-vinyl pyridine and 1 part of (b) a graft copolymer comprising 4-vinyl pyridine (4VP) and vinyl benzyl trimethyl ammonium chloride (TMQ) grafted onto hydroxethyl cellulose (HEC) at a ratio HEC/4VP/TMQ of 2.2/2.2/1, and about 10 mg./ft<sup>2</sup> (about 108 mg./m<sup>2</sup>) of 1,4-butanediol diglycidyl ether cross-linking agent; and

35 4. a decolorizing layer coated at a coverage of about 100 mg./ft<sup>2</sup> (about 1076 mg./m<sup>2</sup>) and comprising 1 part of a tetrapolymer of diacetone acrylamide, methacrylic acid, styrene and butyl acrylate at a ratio of 1/1/0.1/0.1, 0.75 part of Igepal CO-890 nonylphenoxyethylene oxide ethanol and 0.35 part of polyvinyl pyrrolidone.

#### EXAMPLE 2

An image-receiving element was prepared as described in Example 1 except that the copolymer of diacetone acrylamide and methacrylic acid was 1:1.

#### EXAMPLE 3

An image-receiving element was prepared as described in Example 2 except that the ratio of the diacetone acrylamide/methacrylic acid polymer, Igepal CO-890 and polyvinyl pyrrolidone was 1/0.75/0.35.

#### EXAMPLE 4

An image-receiving element was prepared as described in Example 3 except that the neutralizing and timing layers were omitted.

### EXAMPLE 5

An image-receiving element was prepared by coating a transparent subcoated polyethylene terephthalate 4

When the above described image-receiving elements were used in an integral multicolor diffusion transfer process of the Polaroid SX-70 type using the following cyan, magenta and yellow dye developers

**cyan:**



yellow:



**magenta:**



mil (0.1 mm) support with the following layers:

1. an image-receiving layer comprising about 3170 mg/m<sup>2</sup> of a graft copolymer of 2.2 parts 4-vinyl pyridine and 1 part vinyl benzyl trimethyl ammonium chloride on 2.2 parts of hydroxyethyl cellulose and about 43 mg/m<sup>2</sup> of 1,4-butanediol diglycidyl ether; and

2. a decolorizing layer comprising about 1076 mg/m<sup>2</sup> 65 of a mixture of 1 part 1:1 copolymer of diacetone acrylamide and methacrylic acid, 0.75 part Igepal CO-890, and 0.35 part of polyvinyl pyrrolidone.

in a multilayer negative of the type described in said Ser. No. 33,001, using a layer approximately 0.0026 inch thick of a processing composition comprising:

|                                   |          |
|-----------------------------------|----------|
| Water                             | 40.80 g. |
| Potassium hydroxide (100%)        | 4.59 g.  |
| Poly-diacetone acrylamide oxime   | 0.67 g.  |
| Titanium dioxide                  | 48.49 g. |
| Benzotriazole                     | 0.46 g.  |
| 4-aminopyrazolo-(3,4d)-pyrimidine | 0.24 g.  |

-continued

|                                                              |          |
|--------------------------------------------------------------|----------|
| 6-methyl uracil                                              | 0.25 g.  |
| N-2-hydroxyethyl-N,N',N'-tris-carboxymethyl-ethylene diamine | 0.63 g.  |
| Polyethylene glycol<br>(mol. wt. about 4000)                 | 0.38 g.  |
| bis-( $\beta$ -aminoethyl)-sulfide                           | 0.017 g. |
| Colloidal silica<br>(30% dispersion)                         | 0.78 g.  |
| N-phenethyl- $\alpha$ -picolinium bromide                    | 1.07 g.  |
|                                                              | 1.31 g.  |



good multicolor transfer images were obtained. The background provided by the layer of titanium dioxide appeared apparently substantially white to the viewer within 5 to 10 seconds after the processing composition was distributed between the image-receiving element, demonstrating that the decolorizing polyether had been effective. The decolorizing layers were found to be very resistant to rub off and blocking.

Where the image-receiving element does not contain a neutralizing layer and a timing layer, as in Examples 4 and 5 above, these layers were coated in the photosensitive element between the opaque support and the cyan dye developer layer, as described in U.S. Pat. No. 3,573,043 issued Mar. 30, 1971 to Edwin H. Land.

In certain embodiments of this invention, the positive component 32 and the negative component 30 are temporarily laminated to each other so that the decolorizing layer 26 is in optical contact with the outer layer of the negative component 30. This bond should be of such a nature that these layers may be readily separated by the distribution of the processing composition following rupture of the pod 17. A particularly useful method of providing such a temporary lamination is to apply an aqueous solution of a polyethylene glycol, e.g., a polyethylene glycol having a molecular weight of about 6000 such as that commercially available under the tradename "Carbowax 6000" from Union Carbide Corporation. Such uses of polyethylene glycols are disclosed in U.S. Pat. No. 3,793,023 issued Feb. 19, 1974 to Edwin H. Land and to which reference may be made. A particularly useful composition to provide such a temporary lamination is a 50:50 mixture by weight of Carbowax 6000 and Pluronic F-127.

In certain preferred embodiments of this invention, the positive component 32 and the negative component 30 are held in superposed relationship without being temporarily laminated together. In such embodiments

the decolorizing layer also acts to prevent blocking of the positive and negative components in the integral film unit during storage prior to use.

It is well known in the art that for in camera processing the processing composition should include a viscosity-increasing polymer of the type which, when the composition is spread and dried, forms a relatively firm and stable film. High molecular weight polymers are preferred, and include cellulosic polymers such as sodium carboxymethyl cellulose, hydroxyethyl cellulose and hydroxyethyl carboxymethyl cellulose. Another class of useful viscosity-increasing polymers comprises the oxime polymers disclosed and claimed in the pending application of Lloyd D. Taylor, Ser. No. 894,545 filed Apr. 7, 1978 (now U.S. Pat. No. 4,202,694 issued May 13, 1980). Suitable oxime polymers include polydiacetone acrylamide oxime as well as copolymers, e.g., grafts of diacetone acrylamide oxime onto hydroxyethyl cellulose. It has been found that the decolorizing of the optical filter agent immediately adjacent the interface is particularly effective when the concentration of the viscosity-providing polymer is about 1% by weight or less, e.g., about 0.8% by weight as in the above examples.

Neutralizing layers such as the polymeric acid layer are well known in the art and are described in detail, for example, in the above-noted U.S. Pat. Nos. 3,415,644, 3,573,043 and 3,647,437 to which patents reference may be made.

It will be understood that the concentration of the decolorizing agent is such that in the absence of a pH neutralizing mechanism, such as the polymeric acid layer, the decolorizing agent is insufficient to discharge or "clear" all of the optical filter agent present. Thus, if the polymeric acid layer is omitted one observes that the optical filter agent adjacent the processing composition interface is decolorized but the color of the optical filter agent reappears after a period of time, presumably due to later diffusing optical filter agent.

This invention is applicable to a wide variety of photographic processes as will be readily apparent to one skilled in the art. Dye developers are preferred image-providing substances, as indicated above, and constitute an example of initially diffusible dye image-providing substances. Other useful dye image-providing substances include initially diffusible dyes useful as image dyes per se and which couple with the oxidation product of a silver halide developing agent to provide a non-diffusible product, initially diffusible color couplers which couple with the oxidation product of a silver halide developing agent to provide image dyes, initially non-diffusible compounds which react with the oxidation product of a silver halide developing agent, as by coupling or by cross-oxidation, to release a diffusible dye useful as an image dye per se. The final image may be formed as a result of the diffusion transfer of a soluble complex of undeveloped silver halide, in which event the image may be in silver as is well known. In another dye release system a soluble silver complex formed from undeveloped silver halide may be used to effect a cleavage reaction and release a dye or dye intermediate for transfer. Since these image-forming processes are well known and form no part per se of the present invention, it is not necessary to describe them in detail herein.

It will be understood that the transfer image may be positive or negative, with respect to the photographed

subject matter, as a function of the particular image-forming system employed. The silver halide emulsion may be negative-working or positive-working (e.g., internal latent image) as appropriate for the particular imaging system.

For convenience, the disclosures of the aforementioned U.S. Pat. Nos. 3,415,644, 3,575,043 and 3,647,437 are expressly incorporated herein.

Since certain changes may be made in the above product and process without departing from the scope of the invention herein involved, the invention is not intended to be limited thereto but to include variations and modifications obvious to those skilled in the art and which are within the spirit of the invention and the scope of the appended claims.

What is claimed is:

1. An image-receiving element for use in a diffusion transfer process, said image-receiving element comprising, in sequence, a transparent support, an image-receiving layer for a diffusible image-providing material, and a layer adapted to decolorize a pH-sensitive phthalein dye in aqueous alkaline solution, said decolorizing layer comprising a polyoxyalkylene decolorizing agent hydrogen bonded with at least one other polymer.

2. An image-receiving element as defined in claim 1 wherein said diffusible image-providing material is a dye and said image-receiving layer contains a mordant.

3. An image-receiving element as defined in claim 2 wherein said mordant contains quaternary ammonium moieties.

4. An image-receiving element as defined in claim 2 wherein said dye is a dye developer.

5. An image-receiving element as defined in claim 1 wherein said polyoxyalkylene polymer is a wax-like 45 polyoxyethylene polymer.

6. An image-receiving element as defined in claim 5 wherein said polyoxyethylene polymer is

50

55

60



7. An image-receiving element as defined in claim 1 wherein said other polymer is a copolymer of diacetone acrylamide and methacrylic acid.

10 8. An image receiving element as defined in claim 1 wherein said element also includes a neutralizing layer and a timing layer positioned between said support and said image-receiving layer.

15 9. An image-receiving element for use in a diffusion transfer color process, said image-receiving layer comprising, in sequence, a transparent support, an image-receiving layer comprising a mordant for an image dye, and a layer adapted to decolorize a pH-sensitive phthalein dye in aqueous alkaline solution, said phthalein dye including a



30 moiety, said decolorizing layer comprising a mixture of nonylphenol monoether of a polyethylene glycol and a copolymer of diacetone acrylamide and methacrylic acid.

35 10. An image-receiving element as defined in claim 9 wherein said decolorizing layer also includes polyvinyl pyrrolidone.

11. An image-receiving element as defined in claim 9 wherein said decolorizing layer comprises a 1.0/1.0/0.35 to 1.0/0.75/0.35 ratio by weight of a 1:1 copolymer of diacetone acrylamide and methacrylic acid,



and polyvinyl pyrrolidone.

\* \* \* \* \*

65